



US009951475B2

(12) **United States Patent**  
**Cheng et al.**

(10) **Patent No.:** **US 9,951,475 B2**  
(45) **Date of Patent:** **\*Apr. 24, 2018**

(54) **WET END CHEMICALS FOR DRY END  
STRENGTH IN PAPER**

(71) Applicant: **ECOLAB USA INC.**, St. Paul, MN  
(US)

(72) Inventors: **Weiguo Cheng**, Naperville, IL (US);  
**Mei Liu**, Plainfield, IL (US); **Gary S. Furman, Jr.**, St. Charles, IL (US);  
**Robert M. Lowe**, Chicago, IL (US)

(73) Assignee: **ECOLAB USA INC.**, St. Paul, MN  
(US)

(\*) Notice: Subject to any disclaimer, the term of this patent is extended or adjusted under 35 U.S.C. 154(b) by 0 days.

This patent is subject to a terminal disclaimer.

(21) Appl. No.: **15/397,969**

(22) Filed: **Jan. 4, 2017**

(65) **Prior Publication Data**

US 2017/0121909 A1 May 4, 2017

3,269,891 A \* 8/1966 Reynolds ..... D21H 17/34  
162/169

3,284,393 A 11/1966 Vanderhoff et al.

3,409,500 A 11/1968 Strazzins et al.

3,555,932 A 1/1971 Schwerdhofer

3,556,932 A \* 1/1971 Coscia et al. ..... C08B 31/125  
162/166

3,734,873 A 5/1973 Anderson et al.

3,772,076 A 11/1973 Keim

3,821,069 A 6/1974 Wurzburg

RE28,474 E 7/1974 Anderson et al.

RE28,576 E 10/1975 Anderson et al.

3,968,005 A 7/1976 Wurzburg

4,040,900 A 8/1977 Mazzarella et al.

4,493,659 A 1/1985 Iwashita et al.

4,533,434 A 8/1985 Yoshioka et al.

4,603,176 A 7/1986 Bjorkquist et al.

4,605,702 A 8/1986 Guerro et al.

4,657,946 A 4/1987 Rende et al.

4,915,786 A 4/1990 Sweeney

4,919,821 A 4/1990 Fong et al.

4,929,655 A 5/1990 Takeda et al.

4,956,399 A 9/1990 Kozakiewicz et al.

5,006,590 A 4/1991 Takeda et al.

5,147,908 A 9/1992 Floyd et al.

5,281,307 A 1/1994 Smigo et al.

5,324,792 A 6/1994 Ford

5,438,087 A 8/1995 Ikeda et al.

5,474,856 A 12/1995 Tamagawa et al.

5,571,380 A 11/1996 Fallon et al.

5,597,858 A 1/1997 Ramesh et al.

5,597,859 A 1/1997 Hurlock et al.

5,605,970 A 2/1997 Selvarajan

(Continued)

FOREIGN PATENT DOCUMENTS

CA 2176898 C 10/2006  
DE 4426620 A1 2/1995

(Continued)

OTHER PUBLICATIONS

C. O. Au and Thorn, "Applications of Wet-end Paper Chemistry" 1975, Blackie Academic and Professional an Imprint of Chapman Hall, pp. 76-90.\*

Farley, C.E. "Glyoxalated Polyacrylamide Resin," Wet-Strength Resins and Their Application, Chapter 3. Atlanta, GA: TAPPI Press, 1994, pp. 45-61.

Farley, C.E. and R.B. Wasser. "Sizing with Alkenyl Succinic Anhydride," The Sizing of Paper, 2nd Ed. Atlanta, GA: TAPPI Press, 1989, pp. 51-62.

Frberg, S.E. and S. Jones. "Emulsions," Encyclopedia of Chemical Technology, 4th Ed. vol. 9. Published Online Dec. 4, 2000, pp. 393-413.

(Continued)

Primary Examiner — Jose A Fortuna

(74) Attorney, Agent, or Firm — Eric D. Babych; Brinks Gilson & Lione

(57) **ABSTRACT**

The disclosure provides methods and compositions for increasing the dry strength of paper. The invention utilizes a tailored strength agent whose size and shape is tailored to fit into the junction points between flocs of a paper sheet. The strength agents is in contact with the slurry for just enough time to collect at the junction points but not so much that it can migrate away from there.

15 Claims, 5 Drawing Sheets

(56) **References Cited**

U.S. PATENT DOCUMENTS

|             |        |                    |
|-------------|--------|--------------------|
| 2,601,597 A | 6/1952 | Daniel, Jr. et al. |
| 2,982,749 A | 5/1961 | Friedrich et al.   |
| 3,102,064 A | 8/1963 | Wurzburg et al.    |
| 3,233,962 A | 2/1966 | Nelson             |
| 3,234,076 A | 2/1966 | Goldsmith          |

| (56)                  | References Cited |                           |                   |         |                    |             |
|-----------------------|------------------|---------------------------|-------------------|---------|--------------------|-------------|
| U.S. PATENT DOCUMENTS |                  |                           |                   |         |                    |             |
| 5,654,198 A           | 8/1997           | Carrier et al.            | 9,011,643 B2      | 4/2015  | Gu et al.          |             |
| 5,674,362 A           | 10/1997          | Underwood et al.          | 9,034,145 B2      | 5/2015  | Castro et al.      |             |
| 5,785,813 A           | 7/1998           | Smith et al.              | 9,051,687 B2      | 6/2015  | Esser et al.       |             |
| 5,837,776 A           | 11/1998          | Selvarajan et al.         | 9,145,646 B2      | 9/2015  | Benz et al.        |             |
| 5,865,951 A           | 2/1999           | Kawakami et al.           | 9,181,657 B2 *    | 11/2015 | Castro .....       | D21H 17/31  |
| 5,938,937 A           | 8/1999           | Sparapani et al.          | 9,328,462 B2      | 5/2016  | Chen et al.        |             |
| 5,961,782 A           | 10/1999          | Lu et al.                 | 9,347,181 B2 *    | 5/2016  | Lu .....           | D21H 17/43  |
| 5,985,992 A           | 11/1999          | Chen                      | 9,388,533 B2 *    | 7/2016  | Krapsch .....      | D21C 5/02   |
| 6,013,705 A           | 1/2000           | Chen et al.               | 9,506,195 B2 *    | 11/2016 | Chen .....         | D21H 27/002 |
| 6,013,708 A           | 1/2000           | Mallon et al.             | 9,506,202 B2 *    | 11/2016 | Zhao .....         | D21H 17/375 |
| 6,077,394 A           | 6/2000           | Spence et al.             | 9,567,708 B2 *    | 2/2017  | Cheng .....        | D21H 17/375 |
| 6,083,348 A           | 7/2000           | Auhorn et al.             | 9,624,623 B2      | 4/2017  | St. John et al.    |             |
| 6,190,499 B1          | 2/2001           | Oriaran et al.            | 2003/0224945 A1   | 12/2003 | Twu et al.         |             |
| 6,238,521 B1          | 5/2001           | Shing et al.              | 2004/0060677 A1   | 4/2004  | Huang              |             |
| 6,245,874 B1          | 6/2001           | Staib et al.              | 2004/0084162 A1   | 5/2004  | Shannon et al.     |             |
| 6,315,866 B1          | 11/2001          | Sanchez et al.            | 2005/0103455 A1 * | 5/2005  | Edwards .....      | D21F 11/006 |
| 6,348,132 B1          | 2/2002           | Zhang et al.              |                   |         |                    | 162/111     |
| 6,426,383 B1          | 7/2002           | Fong et al.               | 2006/0037727 A1   | 2/2006  | Hagiopol et al.    |             |
| 6,472,487 B2          | 10/2002          | Schroeder et al.          | 2006/0142535 A1   | 6/2006  | Cyr et al.         |             |
| 6,491,790 B1          | 12/2002          | Proverb et al.            | 2006/0162886 A1 * | 7/2006  | Smith .....        | C08F 265/10 |
| 6,592,718 B1          | 7/2003           | Shing et al.              |                   |         |                    | 162/166     |
| 6,610,209 B1          | 8/2003           | Sommese et al.            | 2006/0201645 A1   | 9/2006  | Ito                |             |
| 6,616,807 B1          | 9/2003           | Dyllick-Brenzinger et al. | 2007/0000630 A1   | 1/2007  | Hassler et al.     |             |
| 6,699,359 B1          | 3/2004           | Luu et al.                | 2008/0149287 A1   | 6/2008  | Hagiopol et al.    |             |
| 6,743,335 B2          | 6/2004           | Proverb et al.            | 2008/0196851 A1   | 8/2008  | Hund et al.        |             |
| 6,746,542 B1          | 6/2004           | Lorenck et al.            | 2008/0277084 A1   | 11/2008 | Denowski et al.    |             |
| 6,787,574 B1          | 9/2004           | Farley et al.             | 2008/0308242 A1   | 12/2008 | Lu et al.          |             |
| 6,815,497 B1          | 11/2004          | Luu et al.                | 2009/0025895 A1 * | 1/2009  | Cowman .....       | D21H 23/10  |
| 6,939,443 B2          | 9/2005           | Ryan et al.               |                   |         |                    | 162/162     |
| 7,034,087 B2          | 4/2006           | Hagiopol et al.           | 2009/0107644 A1   | 4/2009  | Cowman et al.      |             |
| 7,119,148 B2          | 10/2006          | Hagiopol et al.           | 2009/0145566 A1   | 6/2009  | Esser et al.       |             |
| 7,125,469 B2          | 10/2006          | Barcus et al.             | 2009/0165978 A1   | 7/2009  | Hagiopol et al.    |             |
| 7,291,695 B2          | 11/2007          | Wei et al.                | 2009/0281212 A1   | 11/2009 | Pawlowska et al.   |             |
| 7,323,510 B2          | 1/2008           | Fischer et al.            | 2010/0193147 A1   | 8/2010  | Ryan et al.        |             |
| 7,455,751 B2          | 11/2008          | Ward et al.               | 2010/0193148 A1   | 8/2010  | McKay et al.       |             |
| 7,488,403 B2          | 2/2009           | Hagiopol et al.           | 2011/0083821 A1   | 4/2011  | Wright             |             |
| 7,550,060 B2          | 6/2009           | Jacobson et al.           | 2011/0112224 A1   | 5/2011  | Borkar et al.      |             |
| 7,615,135 B2          | 11/2009          | Harrington et al.         | 2011/0132559 A1   | 6/2011  | Haehnle et al.     |             |
| 7,641,766 B2          | 1/2010           | St. John et al.           | 2011/0146925 A1   | 6/2011  | Bode et al.        |             |
| 7,641,776 B2          | 1/2010           | Nagar et al.              | 2011/0155339 A1   | 6/2011  | Brungardt et al.   |             |
| 7,683,121 B2          | 3/2010           | Wei et al.                | 2011/0290434 A1 * | 12/2011 | Jehn-Rendu .....   | D21C 9/005  |
| 7,740,743 B2          | 6/2010           | Singh et al.              |                   |         |                    | 162/4       |
| 7,794,565 B2          | 9/2010           | Shannon et al.            | 2012/0035306 A1   | 2/2012  | Ryan et al.        |             |
| 7,863,395 B2          | 1/2011           | Hagiopol et al.           | 2012/0073773 A1   | 3/2012  | Jehn-Rendu et al.  |             |
| 7,897,013 B2          | 3/2011           | Hagiopol et al.           | 2012/0073774 A1   | 3/2012  | Jehn-Rendu et al.  |             |
| 7,914,646 B2          | 3/2011           | Duggirala et al.          | 2012/0103546 A1   | 5/2012  | Maniere            |             |
| 7,938,934 B2          | 5/2011           | Todorovic et al.          | 2012/0103547 A1   | 5/2012  | Grimm et al.       |             |
| 7,972,478 B2          | 7/2011           | Hund et al.               | 2012/0111517 A1   | 5/2012  | Borkar et al.      |             |
| 8,025,924 B2          | 9/2011           | Ohira et al.              | 2012/0186764 A1   | 7/2012  | McKay              |             |
| 8,070,914 B2          | 12/2011          | Ryan et al.               | 2013/0081771 A1   | 4/2013  | Luo et al.         |             |
| 8,088,213 B2          | 1/2012           | Cheng et al.              | 2013/0133847 A1   | 5/2013  | Zhao et al.        |             |
| 8,088,250 B2          | 1/2012           | Cheng et al.              | 2013/0139985 A1   | 6/2013  | Wright             |             |
| 8,288,502 B2          | 10/2012          | Bode et al.               | 2013/0160959 A1   | 6/2013  | Rosencrance et al. |             |
| 8,349,134 B2          | 1/2013           | Esser et al.              | 2013/0192782 A1   | 8/2013  | Benz et al.        |             |
| 8,382,947 B2          | 2/2013           | Skaggs et al.             | 2013/0306261 A1   | 11/2013 | Zhao et al.        |             |
| 8,404,083 B2          | 3/2013           | Haehnle et al.            | 2014/0053996 A1   | 2/2014  | Esser et al.       |             |
| 8,414,739 B2          | 4/2013           | Kimura et al.             | 2014/0060763 A1   | 3/2014  | Bode et al.        |             |
| 8,425,724 B2          | 4/2013           | Ryan et al.               | 2014/0130994 A1   | 5/2014  | St. John et al.    |             |
| 8,444,818 B2          | 5/2013           | Sutman et al.             | 2014/0182799 A1   | 7/2014  | Castro et al.      |             |
| 8,454,798 B2          | 6/2013           | Ban et al.                | 2014/0262091 A1   | 9/2014  | Lu et al.          |             |
| 8,465,623 B2          | 6/2013           | Zhao et al.               | 2014/0284011 A1   | 9/2014  | Krapsch et al.     |             |
| 8,636,875 B2          | 1/2014           | McKay                     | 2014/0336314 A1   | 11/2014 | Benz et al.        |             |
| 8,647,472 B2          | 2/2014           | Cheng et al.              | 2015/0020988 A1   | 1/2015  | St. John et al.    |             |
| 8,696,869 B2          | 4/2014           | Borkar et al.             | 2015/0041088 A1   | 2/2015  | Castro et al.      |             |
| 8,709,207 B2          | 4/2014           | Grimm et al.              | 2015/0041089 A1   | 2/2015  | Castro et al.      |             |
| 8,709,208 B2          | 4/2014           | Zhao et al.               | 2015/0041092 A1   | 2/2015  | Hietaniemi et al.  |             |
| RE44,936 E            | 6/2014           | St. John et al.           | 2015/0059998 A1   | 3/2015  | Zhao et al.        |             |
| 8,747,617 B2          | 6/2014           | Cheng et al.              | 2015/0176206 A1   | 6/2015  | Chen et al.        |             |
| 8,753,480 B2          | 6/2014           | Bode et al.               | 2015/0191875 A1   | 7/2015  | Esser et al.       |             |
| 8,840,759 B2          | 9/2014           | Benz et al.               | 2015/0197893 A1   | 7/2015  | Cheng et al.       |             |
| 8,852,400 B2          | 10/2014          | St. John et al.           | 2015/0204019 A1   | 7/2015  | Wright             |             |
| 8,882,964 B2          | 11/2014          | Zhao et al.               | 2015/0299961 A1   | 10/2015 | Borkar et al.      |             |
| 8,894,817 B1          | 11/2014          | Cheng et al.              | 2016/0097160 A1   | 4/2016  | Castro et al.      |             |
| 8,920,606 B2          | 12/2014          | Wright                    | 2016/0097161 A1   | 4/2016  | Benz et al.        |             |
| 8,999,111 B2          | 4/2015           | Castro et al.             |                   |         |                    |             |

(56)

**References Cited**

## U.S. PATENT DOCUMENTS

2016/0298297 A1\* 10/2016 Borkar ..... D21H 21/20  
 2017/0037574 A1\* 2/2017 Grimm ..... C08F 220/56  
 2017/0121909 A1\* 5/2017 Cheng ..... D21H 17/375

## FOREIGN PATENT DOCUMENTS

|    |                |    |         |
|----|----------------|----|---------|
| EP | 0151994        | A2 | 8/1985  |
| EP | 183466         | B1 | 8/1990  |
| EP | 657478         | A2 | 6/1995  |
| EP | 630909         | B1 | 10/1998 |
| EP | 1195259        | A2 | 4/2002  |
| EP | 1579071        | B1 | 7/2008  |
| JP | H 06-299494    | A  | 10/1994 |
| JP | 2005-001197    | A  | 1/2005  |
| JP | 2008-049688    | A  | 3/2008  |
| JP | 2012-107356    | A  | 6/2012  |
| JP | 05247883       | B2 | 7/2013  |
| WO | WO 1997/05330  | A1 | 2/1997  |
| WO | WO 1997/10387  | A1 | 3/1997  |
| WO | WO 2000/11053  | A1 | 3/2000  |
| WO | WO 2004/061235 | A1 | 7/2004  |
| WO | WO 2004/072376 | A1 | 8/2004  |
| WO | WO 2008/028865 | A2 | 3/2008  |
| WO | WO 2012/007364 | A1 | 1/2012  |
| WO | WO 2013/078133 | A1 | 5/2013  |
| WO | WO 2013/192082 | A1 | 12/2013 |
| WO | WO 2014/078102 | A1 | 5/2014  |

## OTHER PUBLICATIONS

Hercobond Product Analysis (2002), Nalco Chemical Company, one page.

Hunkeler, et al. "Mechanism, Kinetics and Modeling of the Inverse-Microsuspension Homopolymerization of Acrylamide," Polymer. vol. 30, No. 1, 1989, pp. 127-142.

Hunkeler et al. "Mechanism, Kinetics and Modeling of Inverse-Microsuspension Polymerization: 2. Copolymerization of Acrylamide with Quaternary Ammonium Cationic Monomers," Polymer. vol. 32, No. 14, 1991, pp. 2626-2640.

Parez Product Analysis (1999), Nalco Chemical Company, 30 pages.

Smook, Gary A. "Non-fibrous Additives to Papermaking Stock," Handbook for Pulp and Paper Technologists, 2<sup>nd</sup> Ed. Vancouver, BC: Angus Wilde Publications Inc, 1992, pp. 220-227.

St. John, M.R., "Ondeo-Nalco Technical Exchange." Jun. 27, 2002, 5 pages.

EPO Extended European Search Report for EP App. No. 13855150. 2, dated Jun. 15, 2016, 12 pages.

PCT International Search Report and Written Opinion for PCT/ US2015/054064, dated Nov. 30, 2015 (13 pages).

PCT International Search Report and Written Opinion for PCT/ US2015/054069, dated Jan. 22, 2016 (13 pages).

Parez Product Analysis (1999), Nalco Chemical Company, 20 pages.

Nie, Xun-zai, "Papermaking Process," China Light Industry Press, 1999, p. 65, 6 pages, with English Abstract.

"Aego<sup>TM</sup> Sizer F—The PMT Film Size Press: How to improve paper strength properties, surface and machine runnability," TAPPSA Journal, vol. 5 (2013), pp. 38-40.

Biricik, Yagmur, S. Sonmex, and O Ozden, "Effects of Surface Sizing with Starch on Physical Strength Properties of Paper," Asian Journal of Chemistry, vol. 23, No. 7 (2011) pp. 3151-3154.

\* cited by examiner



FIG. 1



**FIG. 2**



FIG. 3



FIG. 4



FIG. 5

WET END CHEMICALS FOR DRY END  
STRENGTH IN PAPER

## BACKGROUND

The invention relates to compositions, methods, and apparatuses for improving dry strength in paper using a process of treating pulp slurry with a combination of strength agents.

As described for example in U.S. Pat. Nos. 8,465,623, 7,125,469, 7,615,135 and 7,641,776 and U.S. patent application Ser. No. 13/962,556, a number of materials function as effective wet-end dry strength agents. These agents can be added to the slurry to increase the tensile strength properties of the resulting sheet. As with retention aids however they must both allow for the free drainage of water from the slurry and also must not interfere with or otherwise degrade the effectiveness of other additives present in the resulting paper product.

Maintaining high levels of dry strength is a critical parameter for many papermakers. Obtaining high levels of dry strength may allow a papermaker to make high performance grades of paper where greater dry strength is required, use less or lower grade pulp furnish to achieve a given strength objective, increase productivity by reducing breaks on the machine, or refine less and thereby reduce energy costs. The productivity of a paper machine is frequently determined by the rate of water drainage from a slurry of paper fiber on a forming wire. Thus, chemistry that gives high levels of dry strength while increasing drainage on the machine is highly desirable.

As described, for example, in U.S. Pat. Nos. 7,740,743, 3,555,932, 8,454,798, and U.S. Patent Application Publication Nos. 2012/0186764, 2012/0073773, 2008/0196851, 2004/0060677, and 2011/0155339, a number of compositions such as glyoxalated acrylamide-containing polymers are known to give excellent dry strength when added to a pulp slurry. U.S. Pat. No. 5,938,937 teaches that an aqueous dispersion of a cationic amide-containing polymer can be made wherein the dispersion has a high inorganic salt content. U.S. Pat. No. 7,323,510 teaches that an aqueous dispersion of a cationic amide-containing polymer can be made wherein the dispersion has a low inorganic salt content. European Patent No. 1,579,071 B1 teaches that adding both a vinylamine-containing polymer and a glyoxalated polyacrylamide polymer gives a marked dry strength increase to a paper product, while increasing the drainage performance of the paper machine. This method also significantly enhances the permanent wet strength of a paper product produced thereby. Many cationic additives, but especially vinylamine-containing polymers, are known to negatively affect the performance of optical brightening agents (OBA). This may prevent the application of this method into grades of paper containing OBA. U.S. Pat. No. 6,939,443, teaches that the use of combinations of polyamide-epichlorohydrin (PAE) resins with anionic polyacrylamide additives with specific charge densities and molecular weights can enhance the dry strength of a paper product. However, these combinations require the use of more than optimal amounts of additives and are sometimes practiced under difficult or cumbersome circumstances. As a result there is clear utility in novel methods for increasing the dry strength of paper.

The art described in this section is not intended to constitute an admission that any patent, publication or other information referred to herein is "prior art" with respect to this invention, unless specifically designated as such. In addition, this section should not be construed to mean that

a search has been made or that no other pertinent information as defined in 37 CFR § 1.56(a) exists.

## BRIEF SUMMARY

To satisfy the long-felt but unsolved needs identified above, at least one embodiment of the invention is directed towards a method of increasing the dry strength of a paper substrate. The method comprises the step of adding a GPAM copolymer to a paper substrate in the wet-end of a papermaking process after the substrate has passed through a screen but before the substrate enters a headbox. The GPAM copolymer may be constructed out of AcAm-AA copolymer intermediates having an average molecular weight of 5-15 kD, and the GPAM copolymer may have an average molecular weight of 0.2-4 MD. In some embodiments, the addition of the GPAM occurs no more than 18 seconds before the substrate enters a headbox. In some embodiments, the GPAM addition occurs no more than 10 seconds before the substrate enters a headbox.

The GPAM may be added subsequent to the addition of an RDF to the paper substrate. The average molecular weight of intermediate for GPAM may be between 5 to 10 kD. The average molecular weight of intermediate for GPAM may be between 6 to 8 kD. The intermediates may have an m-value (FIG. 4) of between 0.03 to 0.20.

The paper substrate may undergo flocculation prior to the GPAM addition which results in the formation of flocs contacting each other at junction points and defining interface regions between the flocs. A majority of the GPAM added may be positioned at junction points and as low as 0% of the GPAM is located within the central 80% of the volume of each formed floc. Essentially no GPAM may be located within the central 80% of the volume of each formed floc.

The paper substrate may comprise filler particles. The paper substrate may have a greater dry strength than a similarly treated paper substrate in which the GPAM was in contact for more than 10 seconds. The paper substrate may have a greater dry strength than a similarly treated paper substrate in which the GPAM was manufactured out of intermediates of greater molecular weight. The paper substrate may have a greater dry strength than a similarly treated paper substrate in which the GPAM had a greater molecular weight.

At least one embodiment of the invention is directed towards a method of increasing the dry strength of a paper substrate. The method comprises the step of adding a strength agent to a paper substrate, wherein: said addition occurs in the wet-end of a papermaking process after the substrate has passed through a screen but no more than 10 seconds before the substrate enters a headbox.

At least one embodiment of the invention is directed towards a method of increasing the dry strength of a paper substrate. The method comprises the step of adding a GPAM copolymer to a paper substrate, wherein: the GPAM copolymer is constructed out of AcAm-AA copolymer intermediates having an average molecular weight of 6-8 kD, the GPAM copolymer has an average molecular weight of 0.2-4 MD.

Additional features and advantages are described herein, and will be apparent from, the following Detailed Description.

BRIEF DESCRIPTION OF THE DRAWING  
FIGURES

A detailed description of the invention is hereafter described with specific reference being made to the drawings in which:

FIG. 1 is an illustration of the distribution of strength agent particles in paper flocs according to the invention.

FIG. 2 is an illustration of one possible example of a papermaking process involved in the invention.

FIG. 3 is an illustration of the distribution of strength agent particles in paper flocs according to the prior art.

FIG. 4 is an illustration of a method of manufacturing a modified GPAM copolymer.

FIG. 5 is an illustration of the distribution of strength agent particles in a single paper floc according to the invention.

For the purposes of this disclosure, like reference numerals in the figures shall refer to like features unless otherwise indicated. The drawings are only an exemplification of the principles of the invention and are not intended to limit the invention to the particular embodiments illustrated.

#### DETAILED DESCRIPTION

The following definitions are provided to determine how terms used in this application, and in particular how the claims, are to be construed. The organization of the definitions is for convenience only and is not intended to limit any of the definitions to any particular category.

“NBSK” means Northern bleached softwood kraft pulp.

“NBHK” means Northern bleached hardwood kraft pulp.

“SW” means softwood pulp.

“HW” means hardwood pulp.

“AA” means acrylic acid.

“AcAm” means acrylamide.

“Wet End” means that portion of the papermaking process prior to a press section where a liquid medium such as water typically comprises more than 45% of the mass of the substrate, additives added in a wet end typically penetrate and distribute within the slurry.

“Dry End” means that portion of the papermaking process including and subsequent to a press section where a liquid medium such as water typically comprises less than 45% of the mass of the substrate, dry end includes but is not limited to the size press portion of a papermaking process, additives added in a dry end typically remain in a distinct coating layer outside of the slurry.

“Surface Strength” means the tendency of a paper substrate to resist damage due to abrasive force.

“Dry Strength” means the tendency of a paper substrate to resist damage due to shear force(s), it includes but is not limited to surface strength.

“Wet Strength” means the tendency of a paper substrate to resist damage due to shear force(s) when rewet.

“Wet Web Strength” means the tendency of a paper substrate to resist shear force(s) while the substrate is still wet.

“Substrate” means a mass containing paper fibers going through or having gone through a papermaking process, substrates include wet web, paper mat, slurry, paper sheet, and paper products.

“Paper Product” means the end product of a papermaking process it includes but is not limited to writing paper, printer paper, tissue paper, cardboard, paperboard, and packaging paper.

“Coagulant” means a water treatment chemical often used in solid-liquid separation stage to neutralize charges of suspended solids/particles so that they can agglomerate, coagulants are often categorized as inorganic coagulants, organic coagulants, and blends of inorganic and organic coagulants, inorganic coagulants often include or comprise aluminum or iron salts, such as aluminum sulfate/choride,

ferric chloride/sulfate, polyaluminum chloride, and/or aluminum chloride hydrate, organic coagulants are often positively charged polymeric compounds with low molecular weight, including but not limited to polyamines, polyquaternaries, polyDADMAC, Epi-DMA, coagulants often have a higher charge density and lower molecular weight than a flocculant, often when coagulants are added to a liquid containing finely divided suspended particles, it destabilizes and aggregates the solids through the mechanism of ionic charge neutralization, additional properties and examples of coagulants are recited in *Kirk-Othmer Encyclopedia of Chemical Technology*, 5th Edition, (2005), (Published by Wiley, John & Sons, Inc.).

“Colloid” or “Colloidal System” means a substance containing ultra-small particles substantially evenly dispersed throughout another substance, the colloid consists of two separate phases: a dispersed phase (or internal phase) and a continuous phase (or dispersion medium) within which the dispersed phase particles are dispersed, the dispersed phase particles may be solid, liquid, or gas, the dispersed-phase particles have a diameter of between approximately 1 and 1,000,000 nanometers, the dispersed-phase particles or droplets are affected largely by the surface chemistry present in the colloid.

“Colloidal Silica” means a colloid in which the primary dispersed-phase particles comprise silicon containing molecules, this definition includes the full teachings of the reference book: *The Chemistry of Silica: Solubility, Polymerization, Colloid and Surface Properties and Biochemistry of Silica*, by Ralph K. Iler, John Wiley and Sons, Inc., (1979) generally and also in particular pages 312-599, in general when the particles have a diameter of above 100 nm they are referred to as sols, aquasols, or nanoparticles.

“Colloidal Stability” means the tendency of the components of the colloid to remain in colloidal state and to not either cross-link, divide into gravitationally separate phases, and/or otherwise fail to maintain a colloidal state its exact metes and bounds and protocols for measuring it are elucidated in *The Chemistry of Silica: Solubility, Polymerization, Colloid and Surface Properties and Biochemistry of Silica*, by Ralph K. Iler, John Wiley and Sons, Inc., (1979).

“Consisting Essentially of” means that the methods and compositions may include additional steps, components, ingredients or the like, but only if the additional steps, components and/or ingredients do not materially alter the basic and novel characteristics of the claimed methods and compositions.

“DADMAC” means monomeric units of diallyldimethylammonium chloride, DADMAC can be present in a homopolymer or in a copolymer comprising other monomeric units.

“Droplet” means a mass of dispersed phase matter surrounded by continuous phase liquid, it may be suspended solid or a dispersed liquid.

“Effective amount” means a dosage of any additive that affords an increase in one of the three quantiles when compared to an undosed control sample.

“Flocculant” means a composition of matter which when added to a liquid carrier phase within which certain particles are thermodynamically inclined to disperse, induces agglomerations of those particles to form as a result of weak physical forces such as surface tension and adsorption, flocculation often involves the formation of discrete globules of particles aggregated together with films of liquid carrier interposed between the aggregated globules, as used herein flocculation includes those descriptions recited in ASTME 20-85 as well as those recited in Kirk-Othmer

Encyclopedia of Chemical Technology, 5th Edition, (2005), (Published by Wiley, John & Sons, Inc.), flocculants often have a low charge density and a high molecular weight (in excess of 1,000,000) which when added to a liquid containing finely divided suspended particles, destabilizes and aggregates the solids through the mechanism of interparticle bridging.

“Flocculating Agent” means a composition of matter which when added to a liquid destabilizes, and aggregates colloidal and finely divided suspended particles in the liquid, flocculants and coagulants can be flocculating agents.

“GCC” means ground calcium carbonate filler particles, which are manufactured by grinding naturally occurring calcium carbonate bearing rock.

“GPAM” means glyoxalated polyacrylamide, which is a polymer made from polymerized acrylamide monomers (which may or may not be a copolymer comprising one or more other monomers as well) and in which acrylamide polymeric units have been reacted with glyoxal groups, representative examples of GPAM are described in US Published Patent Application 2009/0165978.

“Interface” means the surface forming a boundary between two or more phases of a liquid system.

“Papermaking process” means any portion of a method of making paper products from pulp comprising forming an aqueous cellulosic papermaking furnish, draining the furnish to form a sheet and drying the sheet. The steps of forming the papermaking furnish, draining and drying may be carried out in any conventional manner generally known to those skilled in the art. The papermaking process may also include a pulping stage, i.e. making pulp from a lignocellulosic raw material and bleaching stage, i.e. chemical treatment of the pulp for brightness improvement, papermaking is further described in the reference *Handbook for Pulp and Paper Technologists*, 3rd Edition, by Gary A. Smook, Angus Wilde Publications Inc., (2002) and *The Nalco Water Handbook* (3rd Edition), by Daniel Flynn, McGraw Hill (2009) in general and in particular pp. 32.1-32.44.

“Microparticle” means a dispersed-phase particle of a colloidal system, generally microparticle refers to particles that have a diameter of between 1 nm and 100 nm which are too small to see by the naked eye because they are smaller than the wavelength of visible light.

In the event that the above definitions or a description stated elsewhere in this application is inconsistent with a meaning (explicit or implicit) which is commonly used, in a dictionary, or stated in a source incorporated by reference into this application, the application and the claim terms in particular are understood to be construed according to the definition or description in this application, and not according to the common definition, dictionary definition, or the definition that was incorporated by reference. In light of the above, in the event that a term can only be understood if it is construed by a dictionary, if the term is defined by the *Kirk-Othmer Encyclopedia of Chemical Technology*, 5th Edition, (2005), (Published by Wiley, John & Sons, Inc.) this definition shall control how the term is to be defined in the claims.

At least one embodiment of the invention is directed towards a method of increasing the dry strength of a paper substrate by adding a glyoxylated polyacrylamide-acrylic acid copolymer (AGPAM) to a slurry after a retention drainage and formation (RDF) chemical has been added, after the slurry has been passed through a screen, prior to the slurry passing into a headbox wherein the slurry enters the headbox less than 10 seconds after it contacts the AGPAM and the AGPAM is formed from an intermediate whose

molecular weight is less than 15 kD. This process results in exceptionally high dry strength properties.

The invention results in superior performance by doing the exact opposite of what the prior art teaches are best practices. As described, for example, in WO 2008/028865 (p. 6) GPAM intermediate copolymers are expected to require an average molecular weight of at least 25 kD preferably at least 30 kD and the larger size of the intermediates, the better the expected results. For example, U.S. 10 Patent Application Publication No. 2012/0186764 (¶[0021]) states “ . . . the dry strength of the final polymer is theoretically maximized with the highest possible molecular weight of [intermediate] prepolymer . . . ” This teaches that although there is a maximum desired value for size of 15 intermediates, until this maximum is reached, smaller intermediates should perform less well than larger intermediates. In contrast, the invention utilizes a specially sized polymer constructed within a very narrow process window whose intermediates are far smaller than the maximum so should 20 not work well but in fact work better than the prior art says they should.

Similarly the invention uses a very brief residence time while the prior art teaches that one should maximize residence time as much as possible. As can be seen in FIG. 2 in 25 one example of at least a portion of a wet-end of a papermaking process thick stock of pulp (1) is diluted (often with white water) to form thin stock (2). Flocculant is added to the thin stock (3) which then passes through a screen (4), has an RDF (5) added (such as a microparticle/silica material), 30 enters a headbox (6), then passes on to the subsequent portions of the papermaking process such as a Fourdrinier wire/table. The prior art teaches that the longer the contact time between the strength agent and the substrate, more interactions occur and therefore it would be most effective to 35 maximize this contact. As a result strength agents are typically added right at the beginning to the thick stock (1). In contrast in the invention the modified GPAM is added at the last possible moment with only seconds to interact.

Without being limited by a particular theory or design of 40 the invention or of the scope afforded in construing the claims, it is believed that the modified GPAM and the brief residence time allow for a highly targeted application of GPAM which yields a highly unexpected result. As illustrated in FIG. 3, after flocculation the paper substrate 45 consists of flocs (7), (aggregated masses of slurry fibers). These aggregated masses themselves have narrow junction points (8) where they contact each other. Over the prolonged residence time the strength agents (9) tend to disperse widely throughout the flocs. The result is that the flocs 50 themselves have strong integrity but the junction points between the flocs are a weak point between them because they are adjacent to unconnected void regions (10), which define the interface region. As illustrated in FIG. 1, by using a modified GPAM copolymer for the brief residence time the 55 combination of the specific size/shape and the time of contact results in the strength agent not having the time to disperse within the flocs (7) and instead concentrating predominantly at the junction points (8). Because the junction points are the weakest structural point in the floc, this 60 concentration results in a large increase in dry strength properties.

In at least one embodiment the modified GPAM is constructed according to a narrow production window. As 65 illustrated in FIG. 4 AA and AcAm monomers are polymerized to form a copolymer intermediate. The intermediate is then reacted with glyoxal to form the modified GPAM strength agent.

An illustration of possible distribution of GPAM in a floc (7) is shown in FIG. 5. The floc is an irregular shaped mass which has a distinct central point (11). “Central point” is a broad term which encompasses one, some, or all of the center of mass, center of volume, and/or center of gravity of the floc. The central volume (12) is a volume subset of the floc which encompasses the central point (11) and has the minimum distance possible between the central point and all points along the boundary of the central volume (12).

It is understood that because both the floc and the medium they are in are aqueous, over time the GPAM will distribute substantially uniformly. As a result limitations in residence time will result in decreases in distribution of the GPAM to the central volume relative to the outer volume (13) (the volume of the floc outside the central volume) and the interface region. The interface region includes the junction points. In at least one embodiment between >50% to 100% of the added GPAM is located in the interface region. In at least one embodiment between >50% to 100% of the added GPAM is located in the interface region and in the outer volume. In at least one embodiment the central region comprises between 1% and 99% of the overall volume of the floc.

In addition it should be understood that even a marginal alteration of the GPAM distribution from the central volume and/or from the outer volume to the interface region and to the junction points will result in an increase in strength. An alteration in distribution even as low as 1% or lower can be expected to increase the strength effects of the GPAM.

The ratio of AA to AcAm monomers in the intermediate copolymer can be expressed as  $m\text{-value}+n\text{-value}=1$  where  $m\text{-value}$  is the relative amount of polymer structural units formed from AA monomers and  $n\text{-value}$  is the relative amount of polymer structural units formed AcAm monomers.

Copolymer intermediates having specific structural geometry and specific sizes can be formed by limiting the  $m\text{-value}$ . In at least one embodiment the  $m\text{-value}$  is between 0.03 to 0.07 and the resulting copolymer intermediate has a size of 7-9 kD. Because the relative amounts of AcAm provides the binding sites for reaction with glyoxal, the number and proximity of the AcAm units will determine the unique structural geometry that the resulting GPAM will have. Steric factors will also limit how many and which of the AcAm units will not react with glyoxal.

In at least one embodiment the final GPAM product carries four functional groups, Acrylic acid, Acrylamide, mono-reacted acrylamide (one glyoxal reacts with one acrylamide) and di-reacted acrylamide (one glyoxal reacts with two acrylamide). Conversion of glyoxal means how much added glyoxal reacted (both mono or di) with acrylamide. Di-reacted acrylamide creates crosslinking and increases molecular weight of the final product.

In at least one embodiment the final GPAM product has an average molecular weight of around 1 mD. The unique structure of a ~1 mD GPAM constructed out of cross-linked 7-9 kD intermediates for the limited residence time allows for greater dry strength than for the same or greater residence times of: a) a 1 mD GPAM made from larger sized intermediates, b) a 1 mD GPAM made from smaller sized intermediates, and c) a 2-10 mD GPAM.

In at least one embodiment the modified GPAM is added after an RDF has been added to the substrate. RDF functions to retain desired materials in the dry-end rather than having them removed along with water being drained away from the substrate. As a result GPAM is predominantly located at the junction points of fiber flocs.

In at least one embodiment a cationic aqueous dispersion-polymer is also added to the substrate, this addition occurring prior to, simultaneous to, and/or after the addition of the GPAM to the substrate.

5 In at least one embodiment the degree of total glyoxal functionalization ranges from 30% to 70%.

In at least one embodiment the intermediate is formed from one or more additional monomers selected from the list consisting of cationic comonomers including, but are not

10 limited to, diallyldimethylammonium chloride (DADMAC), 2-(dimethylamino)ethyl acrylate, 2-(dimethylamino)ethyl methacrylate, 2-(diethylaminoethyl) acrylate, 2-(diethylamino)ethyl methacrylate, 3-(dimethylamino)propyl acrylate, 3-(dimethylamino)propyl methacrylate, 3-(diethylamino)propyl acrylate, 3-(diethylamino)propyl methacrylate, N-[3-(dimethylamino)propyl]acrylamide, N-[3-(dimethylamino)propyl]methacrylamide, N-[3-(diethylamino)propyl]acrylamide, N-[3-(diethylamino)propyl]methacrylamide, [2-(acryloyloxy)ethyl]trimethylammonium chloride, [2-(methacryloyloxy)ethyl]trimethylammonium chloride, [3-(acryloyloxy)propyl]trimethylammonium chloride, [3-(methacryloyloxy)propyl]trimethylammonium chloride, 3-(acrylamidopropyl)trimethylammonium chloride (APTAC), and 25 3-(methacrylamidopropyl)trimethylammonium chloride (MAPTAC). The preferred cationic monomers are DADMAC, APTAC, and MAPTAC.

In at least one embodiment the cationic aqueous dispersion polymers useful in the present invention are one or 30 more of those described in U.S. Pat. No. 7,323,510. As disclosed therein, a polymer of that type is composed generally of two different polymers: (1) A highly cationic dispersant polymer of a relatively lower molecular weight (“dispersant polymer”), and (2) a less cationic polymer of a 35 relatively higher molecular weight that forms a discrete particle phase when synthesized under particular conditions (“discrete phase”). This invention teaches that the dispersion has a low inorganic salt content.

In at least one embodiment this invention can be applied 40 to any of the various grades of paper that benefit from enhanced dry strength including but not limited to linerboard, bag, boxboard, copy paper, container board, corrugating medium, file folder, newsprint, paper board, packaging board, printing and writing, tissue, towel, and publication. These paper grades can be comprised of any typical pulp fibers including groundwood, bleached or unbleached Kraft, sulfate, semi-mechanical, mechanical, semi-chemical, and recycled.

In at least one embodiment the paper substrate comprises 50 filler particles such as PCC, GCC, and preflocculated filler materials. In at least one embodiment the filler particles are added according to the methods and/or with the compositions described in U.S. patent application Ser. Nos. 11/854, 044, 12/727,299, and/or 13/919,167.

## EXAMPLES

The foregoing may be better understood by reference to the following examples, which are presented for purposes of 60 illustration and are not intended to limit the scope of the invention. In particular the examples demonstrate representative examples of principles innate to the invention and these principles are not strictly limited to the specific condition recited in these examples. As a result it should be understood that the invention encompasses various changes and modifications to the examples described herein and such changes and modifications can be made without departing

from the spirit and scope of the invention and without diminishing its intended advantages. It is therefore intended that such changes and modifications be covered by the appended claims.

The purpose of example 1 and 2 is to demonstrate the effect of addition points of dry strength agent on sheet strength properties.

#### Example 1

The furnish used consisted of 24% PCC, 19% softwood and 57% hardwood. PCC is Albacar HO, obtained from Specialty Mineral Inc. (SMI) Bethlehem, Pa. USA. Both softwood and hardwood are made from dry laps and refined to 400 CSF freeness.

Handsheets are prepared by mixing 570 mL of 0.6% consistency furnish at 1200 rpm in a Dynamic Drainage Jar with the bottom screen covered by a solid sheet of plastic to prevent drainage. The Dynamic Drainage Jar and mixer are available from Paper Chemistry Consulting Laboratory, Inc., Carmel, N.Y. Mixing is started and 18 lb/ton cationic starch Stalok 300 is added after 15 seconds, followed by 0, 2 or 4 lb/ton dry strength agent at 30 seconds, and 1 b/ton (product based) cationic flocculant N-61067 available from Nalco Company, Naperville, Ill. USA) at 45 seconds, followed by 11b/ton active microparticle N-8699 available from Nalco Company, Naperville, Ill. USA at 60 seconds.

Mixing is stopped at 75 seconds and the furnish is transferred into the deckle box of a Noble & Wood handsheet mold. The 8"×8" handsheet is formed by drainage through a 100 mesh forming wire. The handsheet is couched from the sheet mold wire by placing two blotters and a metal plate on the wet handsheet and roll-pressing with six passes of a 25 lb metal roller. The forming wire and one blotter are removed and the handsheet is placed between two new blotters and a metal plate. Then the sheet was pressed at 5.65 MPa under a static press for five minutes. All of the blotters are removed and the handsheet is dried for 60 seconds (metal plate side facing the dryer surface) using a rotary drum drier set at 220° F. The average basis weight of a handsheet is 80 g/m<sup>2</sup>. The handsheet mold, static press, and rotary drum dryer are available from Adirondack Machine Company, Queensbury, N.Y. Five replicate handsheets are produced for each condition.

The finished handsheets are stored overnight at TAPPI standard conditions of 50% relative humidity and 23° C. The basis weight (TAPPI Test Method T 410 om-98), ash content (TAPPI Test Method T 211 om-93) for determination of filler content, and formation, a measure of basis weight unifor-

mity, is determined using a Kajaani® Formation Analyzer from Metso Automation, Helsinki, FI. Basis weight, ash content and Kajaani formation data was listed in Table I. Tensile strength (TAPPI Test Method T 494 om-01) and z-directional tensile strength (ZDT, TAPPI Test Method T 541 om-89) of the handsheets are also tested and listed in Table II. Strength data is strongly dependent on filler content in the sheet. For comparison purpose, all the strength data was also calculated at 20% ash content assuming sheet strength decreases linearly with filler content. The strength data at 20% ash content (AC) was also reported in Table II.

#### Example 2

Example 1 was repeated except that 2 or 4 lb/ton dry strength agent was added 15 seconds after the addition of flocculant N-61067. The handsheet testing results were also summarized in Table I and II.

As shown in Table I and II, addition of strength agent not only increased filler retention, but also increased sheet strength significantly. The effect was even bigger when the dry strength agent was added after flocculant.

#### Example 3

Example 1 was repeated except that the dry strength agent was prepared using different Mw intermediate according to the procedure described in Example A. The handsheet testing results of example 3 was listed in Table III and IV. The results showed intermediate molecular weight affected the performance of dry strength agent significantly. The optimal intermediate molecular weight of dry strength agent was between 6 to 8 thousand Daltons.

#### Example 4

Example 2 was repeated except that dry strength agent was prepared using different Mw intermediate according to the procedure described in Example A. The handsheet testing results of example 4 was listed in Table V and VI. The results showed intermediate molecular weight affected the performance of dry strength agent significantly. The optimal intermediate molecular weight of dry strength agent was between 6 to 8 thousand Daltons. Compared with Example 3, it showed that dry strength agent performed much better when it was added after flocculant. The combination of adding the strength agent after flocculant and choosing optimal intermediate molecular weight for the dry strength agent gave the highest dry strength improvement.

TABLE I

| The effect of GPAM dry strength agent and its addition points on sheet properties |                   |               |              |                    |             |     |               |     |                   |     |
|-----------------------------------------------------------------------------------|-------------------|---------------|--------------|--------------------|-------------|-----|---------------|-----|-------------------|-----|
| Conditions                                                                        | Addition Points   | Dose (lb/ton) | Basis Weight |                    | Ash Content |     | Ash Retention |     | Kajaani Formation |     |
|                                                                                   |                   |               | Dry Strength | Dry Strength (gsm) | Mean        | σ   | Mean          | σ   | Mean              | σ   |
| Reference                                                                         | None              | 0.0           | 74.0         | 0.4                | 16.0        | 0.2 | 61.7          | 1.1 | 109.0             | 1.3 |
| Reference                                                                         | None              | 0.0           | 74.0         | 0.5                | 20.9        | 0.4 | 65.8          | 1.5 | 105.0             | 2.8 |
| Example 1-1                                                                       | Before Flocculant | 2.0           | 77.6         | 0.7                | 19.3        | 0.2 | 77.8          | 0.8 | 99.7              | 2.3 |
| Example 1-2                                                                       | Before Flocculant | 4.0           | 77.6         | 0.5                | 18.9        | 0.4 | 76.3          | 1.8 | 97.5              | 2.1 |
| Example 2-1                                                                       | After Flocculant  | 2.0           | 78.5         | 0.6                | 19.5        | 0.4 | 79.9          | 2.1 | 101.5             | 3.7 |
| Example 2-2                                                                       | After Flocculant  | 4.0           | 78.2         | 0.9                | 19.5        | 0.3 | 79.6          | 2.0 | 101.4             | 1.4 |

TABLE II

| The effect of GPAM dry strength agent and its addition points on sheet strength properties |                   |              |               |              |      |        |           |     |        |                         |     |        |                         |  |  |
|--------------------------------------------------------------------------------------------|-------------------|--------------|---------------|--------------|------|--------|-----------|-----|--------|-------------------------|-----|--------|-------------------------|--|--|
| Conditions                                                                                 | Addition Points   | Dry Strength | Dose (lb/ton) | Dry Strength |      |        | ZDT (kPa) |     |        | Tensile Index (N · m/g) |     |        | TEA (J/m <sup>2</sup> ) |  |  |
|                                                                                            |                   |              |               | Mean         | σ    | 20% AC | Mean      | σ   | 20% AC | Mean                    | σ   | 20% AC |                         |  |  |
| Reference                                                                                  | None              |              | 0.0           | 451.7        | 8.6  | 410.3  | 31.3      | 1.7 | 26.8   | 44.2                    | 5.5 | 32.6   |                         |  |  |
| Reference                                                                                  | None              |              | 0.0           | 401.3        | 9.7  | 410.3  | 25.8      | 1.1 | 26.8   | 30.2                    | 3.1 | 32.6   |                         |  |  |
| Example 1-1                                                                                | Before Flocculant |              | 2.0           | 460.8        | 4.5  | 453.0  | 28.7      | 1.1 | 27.8   | 39.0                    | 4.7 | 36.9   |                         |  |  |
| Example 1-2                                                                                | Before Flocculant |              | 4.0           | 479.8        | 7.1  | 468.1  | 31.8      | 1.1 | 30.5   | 46.9                    | 5.8 | 43.6   |                         |  |  |
| Example 2-1                                                                                | After Flocculant  |              | 2.0           | 468.3        | 13.2 | 463.5  | 31.2      | 1.3 | 30.7   | 46.6                    | 5.1 | 45.2   |                         |  |  |
| Example 2-2                                                                                | After Flocculant  |              | 4.0           | 493.4        | 7.7  | 488.6  | 32.6      | 1.5 | 32.1   | 53.6                    | 2.9 | 52.2   |                         |  |  |

TABLE III

| GPAM samples made out of intermediates with different molecular weight |                         |                      |                 |               |                     |                |              |                      |         |             |  |
|------------------------------------------------------------------------|-------------------------|----------------------|-----------------|---------------|---------------------|----------------|--------------|----------------------|---------|-------------|--|
| sample                                                                 | Intermediate Mw, Dalton | unreacted glyoxal, % | mono-glyoxal, % | di-glyoxal, % | *unreacted amide, % | *mono-amide, % | *di-amide, % | BFV before kill, cps | BFV cps | Final Mw kD |  |
| 6763-129                                                               | 7,400                   | 45                   | 35              | 20            | 73                  | 13             | 14           | 19                   | 10.7    | 1,000       |  |
| 6889-31                                                                | 9,000                   | 53                   | 31              | 16            | 76                  | 12             | 12           | 23                   | 13      | 670         |  |
| 6889-38                                                                | 5,700                   | 46                   | 25              | 29            | 70                  | 9              | 21           | 11.8                 | 6.5     | 2,700       |  |
| 6889-43                                                                | 7,400                   | 46                   | 25              | 29            | 70                  | 9              | 21           | 24                   | 12.8    | 3,000       |  |

TABLE IV

| Dry Strength | Dry Strength  | Basis Weight (gsm) |     |      | Ash Content (%) |      | Ash Retention (%) |      | Kajaani Formation |
|--------------|---------------|--------------------|-----|------|-----------------|------|-------------------|------|-------------------|
| Type         | Dose (lb/ton) | Mean               | σ   | Mean | σ               | Mean | σ                 | Mean | σ                 |
| Reference    | 0.0           | 76.9               | 0.4 | 19.9 | 0.3             | 77.3 | 0.6               | 91.8 | 1.6               |
| Reference    | 0.0           | 75.2               | 1.0 | 24.3 | 0.5             | 97.8 | 1.6               | 92.2 | 3.8               |
| 6763-129     | 2.0           | 78.4               | 0.9 | 21.0 | 0.3             | 82.9 | 2.0               | 81.7 | 3.1               |
| 6763-129     | 4.0           | 78.3               | 1.4 | 21.2 | 0.3             | 83.2 | 2.6               | 81.3 | 4.0               |
| 6889-31      | 2.0           | 78.5               | 0.7 | 21.0 | 0.3             | 82.4 | 1.5               | 80.3 | 5.4               |
| 6889-31      | 4.0           | 78.8               | 0.6 | 21.2 | 0.1             | 84.1 | 0.9               | 77.6 | 1.4               |
| 6889-38      | 2.0           | 77.9               | 0.7 | 20.5 | 0.2             | 79.4 | 0.9               | 84.7 | 1.3               |
| 6889-38      | 4.0           | 78.1               | 0.4 | 20.6 | 0.2             | 81.0 | 0.5               | 84.2 | 1.4               |
| 6889-43      | 2.0           | 77.9               | 0.9 | 20.5 | 0.3             | 79.9 | 1.3               | 83.5 | 2.6               |
| 6889-43      | 4.0           | 78.2               | 0.7 | 21.0 | 0.2             | 82.1 | 0.7               | 82.9 | 4.5               |

TABLE V

| Dry Strength | Dry Strength  | ZDT (kPa) |       | Ash Content |        | Ash Retention |     | TEA (J/m <sup>2</sup> ) |      |     |        |
|--------------|---------------|-----------|-------|-------------|--------|---------------|-----|-------------------------|------|-----|--------|
| Type         | Dose (lb/ton) | (kPa)     | Mean  | σ           | 20% AC | Mean          | σ   | 20% AC                  | Mean | σ   | 20% AC |
| Reference    | 0.0           | 446.3     | 444.0 | 14.6        | 448.7  | 27.7          | 0.5 | 28.0                    | 38.6 | 3.0 | 39.5   |
| Reference    | 0.0           | 376.6     | 387.0 | 15.7        | 448.7  | 23.3          | 1.6 | 28.0                    | 27.0 | 3.4 | 39.5   |
| 6763-129     | 2.0           | 444.0     | 444.3 | 15.9        | 456.7  | 27.2          | 1.1 | 28.1                    | 37.2 | 3.6 | 39.8   |
| 6763-129     | 4.0           | 449.1     | 466.6 | 14.4        | 482.0  | 28.8          | 1.4 | 30.0                    | 42.0 | 3.8 | 45.1   |
| 6889-31      | 2.0           | 413.5     | 437.4 | 16.8        | 450.0  | 26.6          | 1.0 | 27.5                    | 31.8 | 3.8 | 34.4   |
| 6889-31      | 4.0           | 454.6     | 453.8 | 18.9        | 473.3  | 27.3          | 0.6 | 28.7                    | 35.7 | 3.7 | 39.7   |
| 6889-38      | 2.0           | 450.5     | 452.2 | 7.4         | 463.8  | 27.2          | 0.7 | 28.1                    | 36.3 | 3.1 | 38.6   |
| 6889-38      | 4.0           | 473.4     | 477.5 | 9.8         | 490.2  | 28.4          | 0.6 | 29.4                    | 40.6 | 2.7 | 43.2   |
| 6889-43      | 2.0           | 450.4     | 459.8 | 14.1        | 474.0  | 28.2          | 1.5 | 29.3                    | 39.4 | 4.7 | 42.3   |
| 6889-43      | 4.0           | 451.6     | 465.4 | 12.9        | 483.5  | 29.1          | 2.0 | 30.5                    | 40.8 | 5.5 | 44.5   |

TABLE VI

The effect of the molecular weight of intermediate on the performance of GPAM as dry strength agent. GPAM was added after flocculant.

| Dry Strength | Dry Strength  | Basis Weight (gsm) |          | Ash Content (%) |          | Ash Retention (%) |          | Kajaani Formation |          |
|--------------|---------------|--------------------|----------|-----------------|----------|-------------------|----------|-------------------|----------|
| Type         | Dose (lb/ton) | Mean               | $\sigma$ | Mean            | $\sigma$ | Mean              | $\sigma$ | Mean              | $\sigma$ |
| Reference    | 0.0           | 76.7               | 0.6      | 19.8            | 0.3      | 75.9              | 1.6      | 93.8              | 3.4      |
| Reference    | 0.0           | 76.1               | 0.5      | 24.7            | 0.3      | 101.1             | 1.9      | 91.1              | 1.4      |
| 6763-129     | 2.0           | 77.9               | 0.5      | 21.2            | 0.2      | 82.7              | 0.8      | 91.5              | 2.9      |
| 6763-129     | 4.0           | 78.1               | 0.2      | 20.7            | 0.3      | 81.0              | 1.2      | 93.4              | 1.5      |
| 6889-31      | 2.0           | 77.6               | 0.4      | 21.2            | 0.2      | 82.3              | 0.4      | 91.3              | 2.9      |
| 6889-31      | 4.0           | 77.7               | 0.6      | 20.8            | 0.1      | 80.8              | 0.4      | 92.4              | 1.0      |
| 6889-38      | 2.0           | 77.3               | 0.3      | 20.8            | 0.2      | 80.5              | 1.0      | 94.2              | 4.0      |
| 6889-38      | 4.0           | 77.3               | 0.4      | 20.6            | 0.3      | 79.5              | 1.2      | 94.8              | 3.1      |
| 6889-43      | 2.0           | 78.4               | 0.8      | 21.0            | 0.3      | 82.3              | 0.7      | 92.0              | 3.4      |
| 6889-43      | 4.0           | 77.7               | 0.4      | 20.7            | 0.3      | 80.6              | 1.4      | 96.9              | 3.4      |

TABLE VII

The effect of the molecular weight of intermediate on the performance of GPAM as dry strength agent. GPAM was added after flocculant.

| Dry Strength | Dry Strength  | ZDT (kPa) |          |        | Tensile Index (N · m/g) |          |        | TEA (J/m <sup>2</sup> ) |          |        |
|--------------|---------------|-----------|----------|--------|-------------------------|----------|--------|-------------------------|----------|--------|
| Type         | Dose (lb/ton) | Mean      | $\sigma$ | 20% AC | Mean                    | $\sigma$ | 20% AC | Mean                    | $\sigma$ | 20% AC |
| Reference    | 0.0           | 414.1     | 11.3     | 412.3  | 27.5                    | 1.5      | 27.3   | 33.2                    | 4.8      | 32.8   |
| Reference    | 0.0           | 370.3     | 6.4      | 412.3  | 22.9                    | 0.6      | 27.3   | 25.3                    | 2.3      | 32.8   |
| 6763-129     | 2.0           | 462.4     | 12.4     | 473.4  | 29.1                    | 0.4      | 30.2   | 41.2                    | 3.6      | 43.2   |
| 6763-129     | 4.0           | 467.8     | 15.7     | 474.5  | 29.7                    | 1.2      | 30.4   | 39.1                    | 4.4      | 40.3   |
| 6889-31      | 2.0           | 448.1     | 13.4     | 458.9  | 28.6                    | 0.6      | 29.7   | 39.3                    | 1.7      | 41.3   |
| 6889-31      | 4.0           | 466.1     | 22.8     | 473.2  | 29.2                    | 0.4      | 29.9   | 38.2                    | 3.1      | 39.4   |
| 6889-38      | 2.0           | 468.9     | 13.1     | 476.2  | 29.5                    | 0.9      | 30.3   | 40.5                    | 2.7      | 41.9   |
| 6889-38      | 4.0           | 493.0     | 6.0      | 497.9  | 32.1                    | 1.1      | 32.6   | 48.2                    | 3.8      | 49.1   |
| 6889-43      | 2.0           | 463.6     | 6.7      | 472.6  | 29.1                    | 1.2      | 30.0   | 40.2                    | 3.8      | 41.8   |
| 6889-43      | 4.0           | 488.7     | 8.5      | 495.3  | 30.2                    | 1.6      | 30.9   | 43.2                    | 4.3      | 44.4   |

The data demonstrates that both using GPAM of an especially small size and/or limiting the residence time to extremely short periods of time results in unexpected increases in paper strength. For example when a large intermediate GPAM was used with a long residence time the resulting ZDT strength was 463.8 kPa. Under the same conditions a smaller intermediate GPAM resulted in ZDT of 483.5 kPa and a smaller intermediate GPAM with a short residence time resulted in ZDT of 495.3 kPa. Thus by doing the opposite of what the prior art teaches, greater strength can be achieved.

As previously stated, in at least one embodiment utilizing specially sized intermediates produced within in a very narrow process window results in better than expected results. Representative procedures used to produce/use those intermediates are shown in example A below.

#### Example A

##### 6763-129

Representative procedure for the synthesis of polyacrylamide-acrylic acid copolymer

Intermediate A: To a 1 L reaction flask equipped with a mechanical stirrer, thermocouple, condenser, nitrogen purge tube, and addition port was added 145.33 g of water. It was then purged with N<sub>2</sub> and heated to reflux. Upon reaching the desired temperature (~95-100° C.), 22.5 g of a 20% aqueous solution of ammonium persulfate (APS) and 55.36 g of a 25% aqueous solution of sodium meta-bisulfite (SMBS) were added to the mixture through separate ports over a

40 period of 130 min. Two minutes after starting the initiator solution additions, a monomer mixture containing 741.60 g of 51.2% acrylamide, 20.29 g of acrylic acid, 11.42 g of water, 0.12 g of EDTA, and 3 g of 50% sodium hydroxide was added to the reaction mixture over a period of 115 minutes. The reaction was held at reflux for an additional hour after APS and SMBS additions. The mixture was then cooled to room temperature providing the intermediate product as a 40% actives, viscous and clear to amber solution. It had a molecular weight of about 7,400 g/mole.

45 Representative procedure for glyoxalation of polyacrylamide-acrylic acid:

The intermediate product A (70.51 g) prepared above and 50 water (369.6 g) were charged into a 500-mL tall beaker at room temperature. The pH of the polymer solution was adjusted to 8.8-9.2 using 1.4 g of 50% aqueous sodium hydroxide solution. The reaction temperature was set to 55 24-26° C. Glyoxal (21.77 g of a 40% aqueous solution) was added over 15-45 min, pH of the resulting solution was then adjusted to 9-9.5 using 10% sodium hydroxide solution (3.5 g). The brookfield viscosity (Brookfield Programmable DV-E Viscometer, #1 spindle @ 60 rpm, Brookfield Engineering Laboratories, Inc, Middleboro, Mass.) of the mixture was about 3-4 cps after sodium hydroxide addition. The pH of the reaction mixture was maintained at about 8.5 to 9.5 at about 24-26° C. with good mixing (more 10% sodium hydroxide solution can be added if necessary). The Brookfield viscosity (BFV) was measured and monitored every 15-45 minutes and upon achieving the desired viscosity increase of greater than or equal to 1 cps (4 to 200 cps,

## 15

>100,000 g/mole) the pH of the reaction mixture was decreased to 2-3.5 by adding sulfuric acid (93%). The rate of viscosity increase was found to be dependent on the reaction pH. The higher the pH of the reaction, the faster the rate of viscosity increase. The product was a clear to hazy, colorless to amber, fluid with a BFV greater than or equal to 4 cps. The resulting product was more stable upon storage when BFV of the product was less than 40 cps, and when the product was diluted to lower actives. The product can be prepared at higher or lower percent total actives by adjusting the desired target product viscosity. For sample 6889-129, it has a BFV of 10.7 cps, active concentration of 7.69% (total glyoxal and polymer), and molecular weight of about 1 million g/mole.

6889-31

Intermediate B was synthesized following similar process as described for intermediate A except that a different chain transfer agent (sodium hypophosphite) was used. The final product has an active concentration of 36%. It is a viscous and clear to amber solution, and had a molecular weight of about 9,000 g/mole.

6889-31 was synthesized following similar process as described for 6763-129 except that intermediate B was used. The final product has a BFV of 13.2 cps, active concentration of 7.84% (total glyoxal and polymer), and molecular weight of about 670,000 g/mole.

6889-38

Intermediate C was synthesized following similar process as described for intermediate A except that sodium formate and sodium hypophosphite were used as the chain transfer agent. The final product has an active concentration of 36%. It is a viscous and clear to amber solution, and had a molecular weight of about 5,700 g/mole.

6889-38 was synthesized following similar process as described for 6763-129 except that intermediate C was used. The final product has a BFV of 6.5 cps, active concentration of 7.84% (total glyoxal and polymer), and molecular weight of about 2.7 million g/mole.

6889-43

Intermediate D was synthesized following similar process as described for intermediate A except that different chain transfer agent (sodium hypophosphite) was used. The final product has an active concentration of 36% actives. It is a viscous and clear to amber solution, and had a molecular weight of about 7,400 g/mole.

6889-43 was synthesized following similar process as described for 6763-129 except that intermediate D was used. The final product has a BFV of 12.8 cps, active concentration of 7.83% (total glyoxal and polymer), and molecular weight of about 3 million g/mole.

Next a series of tests were performed to demonstrate the effectiveness of the invention on tissue or towel grade paper. Descriptions of methods, apparatuses, and compositions in which the invention can be applied to tissue or towel grade paper include, but are not limited to, those mentioned in U.S. Pat. Nos. 8,753,478, 8,747,616, 8,691,323, 8,518,214, 8,444,812, 8,293,073, 8,021,518, 7,048,826, and 8,101,045, and U.S. Patent Application Publication Nos.: 2014/0110071, 2014/0069600, 2013/0116812, and 2013/0103326.

## Experimental Conditions—

Two thick stock fiber slurries were prepared from NBHK and NBSK dry laps, respectively and were treated according to a narrow process window. The SW dry lap was slushed in a Dyna Pulper for 33 minutes and had a consistency of 3.6% and a CSF of 683 mL. Likewise the HW dry lap was slushed in a Dyna Pulper for 23 minutes and had a consistency of

## 16

3.4% and a CSF of 521 mL. These thick stocks were combined in a ratio of 70/30 HW/SW to prepare a 0.5% consistency thin stock having a pH of 7.9. Tap water was used for dilution. Laboratory handsheets were prepared from the thin stock, using a volume of 500 mL to produce a target basis weight sheet of 60 g/m<sup>2</sup> on a Nobel and Wood sheet mold. The forming wire used was 100 mesh. Prior to placing the 500 mL of thin stock in the handsheet mold, the stock was treated with additives according to the timing scheme shown below. Additive dosing occurred in a Britt Jar with mixing at 1200 rpm.

TABLE VIII

|             | 15 | Time (sec) |         |       |      |    |
|-------------|----|------------|---------|-------|------|----|
|             |    | 0          | 15      | 30    | 45   | 60 |
| Example 5-1 | WS | DA         | AF      |       | stop |    |
| Example 5-2 | WS | AF         | DA      |       | stop |    |
| Example 5-3 | WS | AF         | DA      | MP    | stop |    |
| Example 5-4 | WS | AF         | DA + MP |       | stop |    |
| Example 6-1 | WS | DA         | CF      |       | stop |    |
| Example 6-2 | WS | CF         | DA      |       | stop |    |
| Example 6-3 | WS | CF         | DA      | N8699 | stop |    |
| Example 6-4 | WS | CF         | DA + MP |       | stop |    |
| Reference   | WS |            |         |       | stop |    |

The additives and dosing levels can be further classified as follows:

WS is one or more commercially available wet strength resins having 25% solids; dosed at 15 lb/T actives/dry fiber basis.

DA is one or more commercially available anionic GPAM strength resins; dosed at 4 lb/T actives/dry fiber basis.

DC is one or more commercially available cationic GPAM strength resins; dosed at 4 lb/T actives/dry fiber basis.

DS refers to the applicable DA or DC strength agent of the respective example

AF is one or more commercially available anionic flocculants; dosed at 1 lb/T product/dry fiber basis.

MP is one or more commercially available anionic silica microparticles; dosed at 1 lb/T actives/dry fiber basis.

CF is one or more commercially available cationic flocculants; dosed at 1 lb/T product/dry fiber basis.

45 The sheets were couched from the wire and wet pressed in a roll press at a pressure of 50 lb/in<sup>2</sup>. The pressed sheets were then dried on an electrically heated drum dryer having a surface temperature of 220° F. Finally, the sheets were oven cured at 105° C. for 10 minutes, and then conditioned in a controlled temperature (23° C.) and humidity (50%) room for 24 hours prior to testing.

55 Five handsheets were prepared for each condition evaluated. The sheets were measured for basis weight, dry tensile, wet tensile and formation. Tensile measurements given in the examples are the average of ten tests, and the tensile index was calculated by dividing by the sheet basis weights. Formation measurements given in the examples are the average of five tests. CI refers to the 95% confidence interval calculated from the individual measurements.

## 60 Example 5—Anionic Flocculant with Anionic Dry Strength

65 This example shows the effect of changing the order of addition of an anionic flocculant and anionic dry strength. A higher dry and wet tensile index is indicated when the dry strength is added after the flocculant (compare Ex. 5-1 vs.

5-2). Likewise, addition of the microparticle after the dry strength maintains this increased performance (compare Ex. 5-1 vs. 5-3 and 5-4).

TABLE IX

| Conditions  | Additives given in order of addition | Kajaani Formation |        |
|-------------|--------------------------------------|-------------------|--------|
|             |                                      | Index             | 95% CI |
| Reference   | WS                                   | 103.7             | 2.1    |
| Example 5-1 | WS/DS/AF                             | 96.0              | 5.3    |
| Example 5-2 | WS/AF/DS                             | 96.7              | 3.0    |
| Example 5-3 | WS/AF/DS/MP                          | 100.1             | 1.7    |
| Example 5-4 | WS/AF/DS + MP                        | 98.4              | 2.2    |

TABLE X

| Conditions  | Dry Tensile<br>(Nm/g) |        | Wet Tensile<br>(Nm/g) |        | Wet/Dry<br>(%) |        |
|-------------|-----------------------|--------|-----------------------|--------|----------------|--------|
|             | Index                 | 95% CI | Index                 | 95% CI | Value          | 95% CI |
| Reference   | 35.2                  | 2.5    | 8.4                   | 0.5    | 24.1           | 1.5    |
| Example 5-1 | 37.8                  | 1.9    | 9.3                   | 0.4    | 24.5           | 0.8    |
| Example 5-2 | 38.3                  | 3.0    | 9.9                   | 0.4    | 26.0           | 1.6    |
| Example 5-3 | 39.5                  | 2.0    | 9.6                   | 0.5    | 24.4           | 1.6    |
| Example 5-4 | 39.7                  | 1.9    | 9.3                   | 0.7    | 23.5           | 1.5    |

Example 6—Cationic Flocculant with Anionic Dry Strength

This example shows the effect of changing the order of addition of a cationic flocculant and anionic dry strength. Again a higher dry and wet tensile index is indicated when the dry strength is added after the flocculant (compare Ex. 2-1 vs. 2-2).

TABLE XI

| Conditions  | Additives given in order of addition | Kajaani Formation |        |
|-------------|--------------------------------------|-------------------|--------|
|             |                                      | Index             | 95% CI |
| Reference   | WS                                   | 103.7             | 2.1    |
| Example 6-1 | WS/DS/CF                             | 99.1              | 3.1    |
| Example 6-2 | WS/CF/DS                             | 98.5              | 3.1    |
| Example 6-3 | WS/CF/DS/MP                          | 99.0              | 3.6    |
| Example 6-4 | WS/CF/DS + MP                        | 98.0              | 3.9    |

TABLE XII

| Conditions  | Dry Tensile<br>(Nm/g) |        | Wet Tensile<br>(Nm/g) |        | Wet/Dry<br>(%) |        |
|-------------|-----------------------|--------|-----------------------|--------|----------------|--------|
|             | Index                 | 95% CI | Index                 | 95% CI | Value          | 95% CI |
| Reference   | 35.2                  | 2.5    | 8.4                   | 0.5    | 24.1           | 1.5    |
| Example 6-1 | 36.8                  | 2.4    | 9.0                   | 0.3    | 24.7           | 2.0    |
| Example 6-2 | 41.2                  | 2.2    | 10.1                  | 0.5    | 24.6           | 1.1    |
| Example 6-3 | 36.1                  | 2.3    | 9.2                   | 0.6    | 25.6           | 2.0    |
| Example 6-4 | 38.3                  | 2.2    | 9.8                   | 0.5    | 25.6           | 1.4    |

The data demonstrates that adding the anionic GPAM following the flocculant within a very narrow process window resulted in a higher strength value which was most apparent in Example 6-2.

While this invention may be embodied in many different forms, there are described in detail herein specific preferred embodiments of the invention. The present disclosure is an exemplification of the principles of the invention and is not

intended to limit the invention to the particular embodiments illustrated. All patents, patent applications, scientific papers, and any other referenced materials mentioned herein are incorporated by reference in their entirety. Furthermore, the invention encompasses any possible combination of some or all of the various embodiments mentioned herein, described herein and/or incorporated herein. In addition the invention encompasses any possible combination that also specifically excludes any one or some of the various embodiments mentioned herein, described herein and/or incorporated herein.

The above disclosure is intended to be illustrative and not exhaustive. This description will suggest many variations and alternatives to one of ordinary skill in this art. All these alternatives and variations are intended to be included within the scope of the claims where the term "comprising" means "including, but not limited to". Those familiar with the art may recognize other equivalents to the specific embodiments described herein which equivalents are also intended to be encompassed by the claims.

All ranges and parameters disclosed herein are understood to encompass any and all subranges subsumed therein, and every number between the endpoints. For example, a stated range of "1 to 10" should be considered to include any and all subranges between (and inclusive of) the minimum value of 1 and the maximum value of 10; that is, all subranges beginning with a minimum value of 1 or more, (e.g. 1 to 6.1), and ending with a maximum value of 10 or less, (e.g. 2.3 to 9.4, 3 to 8, 4 to 7), and finally to each number 1, 2, 3, 4, 5, 6, 7, 8, 9, and 10 contained within the range. All percentages, ratios and proportions herein are by weight unless otherwise specified.

This completes the description of the preferred and alternate embodiments of the invention. Those skilled in the art may recognize other equivalents to the specific embodiment described herein which equivalents are intended to be encompassed by the claims attached hereto.

The invention claimed is:

1. A method of increasing the strength of a paper substrate, the method comprising in order:
  - adding a cationic wet strength agent to a paper substrate,
  - adding a flocculating agent to the paper substrate, and
  - adding a glyoxalated polyacrylamide (GPAM) copolymer to the paper substrate, wherein addition of GPAM occurs in the wet-end of a papermaking process after the substrate has passed through a screen but before the substrate enters a headbox.
2. The method of claim 1, wherein the GPAM copolymer is constructed out of acrylamide-acrylic acid (AcAm-AA) copolymer intermediates having an average molecular weight of 5-15 kD, the GPAM copolymer has an average molecular weight of 0.2-4 mD.
3. The method of claim 2, wherein the AcAm-AA copolymer intermediates have an average molecular weight of 5.7-9 kD.
4. The method of claim 2, wherein the intermediates have an m-value of between 0.03 to 0.20, wherein the m-value is a relative amount of polymer structural units formed from AA.
5. The method of claim 1, wherein the GPAM copolymer has an average molecular weight of 0.6-3 mD.
6. The method of claim 1, wherein a retention, drainage, and formation (RDF) chemical is added to the paper substrate before the GPAM.
7. The method of claim 6, wherein the RDF chemical comprises silica.

**19**

**8.** The method of claim 1, wherein the paper substrate undergoes flocculation prior to the GPAM addition, which results in the formation of flocs contacting each other at junction points.

**9.** The method of claim 8, wherein a majority of the GPAM added is positioned at junction points and as low as 0% of the GPAM is located within the central 80% of the volume of each formed floc.

**10.** The method of claim 8, wherein substantially no GPAM is located within the central 80% of the volume of each formed floc.

**11.** The method of claim 1, wherein the paper substrate comprises filler particles.

**12.** The method of claim 1, wherein the paper substrate has a greater dry strength than a similarly treated paper substrate in which the GPAM was in contact for more than 18 seconds.

**13.** The method of claim 1, wherein the paper substrate has a greater dry strength than a similarly treated paper substrate in which the GPAM was manufactured out of intermediates of greater molecular weight.

**14.** The method of claim 1, wherein the paper substrate has a greater dry strength than a similarly treated paper substrate in which the GPAM had a greater molecular weight.

**15.** The method of claim 1, wherein the GPAM copolymer comprises from about 30% to about 70% glyoxal functionalization.

**20**

\* \* \* \* \*